

## UNITED STATES PATENT OFFICE

1,954,407

## CASE HARDENING

John J. Egan, Brooklyn, N. Y., assignor to Electro  
Metallurgical Company, a corporation of West  
Virginia

No Drawing. Application August 11, 1931,  
Serial No. 556,464

3 Claims. (Cl. 148—17)

My invention relates to the production of hard wear-resistant cases or surface layers on ferrous materials by the carbonizing process, referring more particularly to an improved method of producing such cases.

5 The production of carbon-enriched cases on ferrous materials by the surface-carbonizing process is well known. In this process the surface portions of low-carbon steel are enriched with carbon by the action at elevated temperatures of various carbonaceous materials. In order to secure proper penetration of carbon, the materials must be maintained at an elevated temperature for a number of hours, which involves considerable expense. A method which

10 would reduce the time required to produce a case of given depth would result in savings not only in the cost of heating, but also in the cost of apparatus involved.

15 It is the object of my invention to accelerate and intensify the action of gaseous carbonizing agents on ferrous materials, so as to reduce materially the time required to produce a case of given hardness or depth. This object I have attained by the application of my discovery that

20 electrical influences which tend to ionize the gaseous environment of the articles being treated so accelerate and intensify the carbonizing reaction that cases of given depth and hardness may be produced in much less than the usual time. The ionizing influence may be generated by an arc, spark, corona, or other form of electrical discharge in the gaseous environment.

According to the preferred form of my invention, the articles to be treated are placed in a suitable chamber containing a gaseous carbonizing agent or agents, and an electrical discharge is caused to take place within the chamber, preferably in close proximity to the surface of the article. The customary carbonizing temperature is maintained and the discharge is continued throughout the entire time of heating. Suitable electrodes across which the discharge may be drawn can easily be inserted into the chamber. A spark such as that generated at an ordinary internal combustion engine spark plug is an especially convenient form of discharge for this purpose. With one or more spark plugs discharging within the gaseous environment of the article I have been able to produce on typical carbonizing steels cases from two to six times as deep as those produced in the same time and at the same temperature in the absence of the ionizing influence. The improvement secured by the use of my method depends somewhat on the type of steel and the carbonizing agent used, but my invention gives beneficial effects of appreciable magnitude on any carbonizing steel or with any gaseous carbonizing agent.

60 Tests which I have made demonstrate clearly

the acceleration which results from the use of my invention. For example, a cold rolled low-carbon steel treated for 2½ hours with illuminating gas at 915° C. formed a carbonized case 0.02 inches deep when a spark was used in the treating chamber, while without the spark a treatment for 2½ hours at 915° C. in illuminating gas formed a case only 0.005 inches deep, as was to be expected from general experience in the art. Using the same steel and treating for 2½ hours at 915° C. in an atmosphere of propane, the corresponding depths of cases were found to be 0.06 inches in the presence of a spark within the chamber and only 0.01 inches in the absence of an ionizing influence.

75 Further tests which I have made show that the principle of my invention may be applied with beneficial results on any carbonizing steel and in any carbonizing atmosphere, and with the use of any of the usual carbonizing temperatures. 80 Therefore I do not wish to be limited to or by the specific examples which I have disclosed herein, or to the preferred form of my invention. I wish to be limited only by the prior art and the appended claims.

85 I claim:

1. The method of carbonizing ferrous articles which comprises heating the articles in a chamber containing a carbonizing gas while maintaining an ionizing electrical discharge in close proximity to the surface of said articles, the discharge providing no material portion of the heat required to maintain the articles at carbonizing temperatures.

90 2. The method of producing carbon-enriched surface portions on at least part of a low-carbon ferrous article which comprises heating the article in a chamber containing propane; while maintaining in close proximity to the surface of said article an ionizing electrical discharge, which provides no material portion of the heat required to maintain the articles at carbonizing temperatures.

95 3. The method of producing carbon-enriched surface portions on at least part of a ferrous article which comprises heating said portions in the presence of a carbonizing gas while maintaining in close proximity to the heated portions at least one of the following ionizing electrical discharges: arc, spark, corona, the discharge providing no material portion of the heat required to maintain the articles at carbonizing temperatures.

105 JOHN J. EGAN.

110

115

120